

July 7, 1936.

C. W. DAKE

2,046,369

BRAKE DRUM

Original Filed Jan. 15, 1934



Fig. 1.



Fig. 2.

Inventor  
Charles W. Dake  
By Livrance and  
Van Antwerp  
Attorneys

## UNITED STATES PATENT OFFICE

2,046,369

## BRAKE DRUM

Charles W. Dake, Grand Haven, Mich., assignor  
to Campbell, Wyant & Cannon Foundry Com-  
pany, Muskegon Heights, Mich., a corporation  
of Michigan

Original application January 15, 1934, Serial No.  
706,693. Divided and this application May 14,  
1934, Serial No. 725,613

3 Claims. (Cl. 188—218)

This invention relates to a brake drum.

More particularly, this application claims the  
brake drum as an article and is a division of my  
patent granted December 11, 1934, No. 1,983,839.

5 One object of this invention is to economically  
produce a brake drum which will be efficient in  
action. That is, the braking surface is non-porous  
and free from pitting or other defects and  
the outer periphery or the portion adjacent to the  
10 braking band is of stronger metal as will be un-  
derstood from the following specification.

An understanding of the invention and of the  
various objects enumerated, as well as others not  
15 at this time stated, may be had from the follow-  
ing description, taken in connection with the  
accompanying drawing, in which,

Fig. 1 is a vertical section taken diametrically  
of an annular mold in which the drum, ring or  
20 flange is cast, the interior of the mold conform-  
ing to the desired exterior form of the brake  
drum flange.

Fig. 2 is a section taken centrally through a  
brake drum produced in accordance with the  
present invention.

25 Like reference characters refer to like parts  
in the different figures of the drawing.

One form of apparatus with which the mold  
is used and by means of which the casting is  
30 formed is shown in Fig. 1. It includes a revolu-  
ble spindle 10 having an annular flask 11 mounted  
thereon and a mold 12 is positioned in the flask  
11. The upper part of the flask member 11 is  
undercut as shown and retaining segments 13  
35 hold the mold 12 in place.

35 A locating post 14 is provided interiorly of the  
spindle 10 and locates the distributor 15 in posi-  
tion as clearly shown in Fig. 1. The molten  
metal 16, indicated in dotted lines in Fig. 1, is  
40 poured from the ladle 17 and contacts against  
the beveled edge of the distributor 15 and then  
enters the mold 12. As shown, the face of the  
mold 12 is corrugated to form ribs upon the brake  
drum indicated generally by the numeral 20.

45 The molten metal poured into the mold is an  
alloy consisting preferably principally of two  
metal constituents. An example may be fur-  
nished by an alloy of iron and copper. The metal  
in a molten state and, preferably heated consider-  
50 ably above its melting temperature, is poured into  
the rotating mold. Through centrifugal action  
the metal rises against and covers the inner sub-  
stantially vertical face of the mold. It fills all  
55 of the grooves and depressions in the inner sur-  
face of the mold. The shaft 10 and the flask 11  
attached thereto are rotated at high speed. A

peripheral speed of the molten metals of sub-  
stantially 3000 feet per minute has the effect of  
causing the two metals of different specific grav-  
ity, cast iron and copper, to separate, the heavier  
metal going to the outside. If the speed is in-  
creased to a peripheral speed of the metals of  
5 5000 feet per minute, there will be a very nearly  
complete separation of the copper and cast iron,  
whereby there will be produced a casting, the  
inner annular portion 24 of which is of cast iron, 10  
the outer annular portion 25, including the pro-  
jecting annular ribs thereon, of copper and at the  
junction of the two, indicated by dotted lines at  
15 26, there will be no sharp separation of the metals  
but an intermediate zone where the two are inti- 15  
mately mingled. This zone follows the outer  
contour of the drum and consequently has a cen-  
tral bulge thereon. This bulge provides a rein-  
forcing rib for the ring. Also, it increases the  
rate of heat transfer outwardly through the ring 20  
inasmuch as it increases the surface contact be-  
tween the cast iron and the copper and the  
rate of heat transfer is dependent upon the size  
of the contacting surfaces. In practice the quan-  
tity of copper used should not exceed 15% of 25  
the mass of metal.

The temperature of the molten metal may  
range from 2300° F. to 3000° F. when an alloy of  
cast iron and copper is used as described. Copper  
melts at 1981.4° F. and cast iron from 1900° to 30  
2200° F., depending upon the composition of the  
cast iron. At 2300° F. all of the metal will be  
melted, and heated somewhat above melting tem-  
perature. Preferably, the temperature should be  
sufficiently above the melting point that the 35  
molten metals will remain in a freely fluid state  
for a period of time during the operation such  
that there can be ready separation under the  
centrifugal forces operating upon them, and there  
will not be too rapid a solidification such that any 40  
solidifying or thickening of the molten metals  
would interrupt the separation. In addition any  
gases, impurities, slag or the like should be en-  
abled to pass with freedom through the molten  
metal to the inner surface of the ring casting 45  
and thus eliminate any possibility of defects, such  
as porosity or trapped slag or other impurities in  
the cast iron which would detrimentally affect  
the braking surface of the cast iron after it has  
been machined at the inner curved surface of the 50  
casting produced. For these reasons the use of  
a temperature in pouring but little above the  
temperature at which the metals will be all melted  
is to be avoided, and considerably higher than  
mere melting temperature used. 55

The drum thus produced, using cast iron and copper as the metals, has an inner braking face of cast iron and an outer supporting shell of copper which is not brittle like cast iron but has the property of toughness and strength. The brake drum ring produced therefore combines the desired soft, yet positive braking characteristics of cast iron without the necessity of using an undue weight of metal which would be needed if cast iron alone was used, the copper shell providing the necessary toughness and tensile strength to insure the drum against breaking under shock.

As previously described the extent of separation is governed by the rotative speed. The higher speeds, which produce a peripheral speed of substantially 5000 lineal feet per minute of the molten metal, are better than the lower speed of 3000 lineal feet per minute peripheral speed because of the greater separation of the cast iron and copper; and there will be proportionally greater or less separation as the speed is increased or diminished. What is the best speed for the particular article being manufactured may be determined by test and experience.

It is to be understood that while a specific example of two metals like cast iron and copper has been given the invention is in nowise limited to the use of such two metals alone. Other metals may be used together, that is, preferably other metals than copper with cast iron for brake drum purposes. And for other purposes wherein the inner material does not necessarily have to be of cast iron other suitable metal for the desired purpose may be used in its place. Such different metals with their differing specific gravities will require a speed of rotation in correspondence with the differences in specific gravity. If the two metals are nearer together in specific gravity than are copper and cast iron, the speed of rotation will need to be increased. If they are farther apart in specific gravity the speed of rotation can be reduced so as to get the desired effective separation. It is further to be understood that while the temperature should preferably be considerably above the temperature at which the metals will be wholly molten, when cast iron is used as

one of the metals and the other metal has a melting point like copper of substantially 2000° F. the composition of the cast iron will be controlling as to its melting point, and the temperature of the composite mixture when poured into the mold can be lower for a low temperature melting cast iron than for a high temperature melting cast iron. Also a high phosphorus content in cast iron renders the same much more fluid than one using low phosphorus content and the temperature to which the composite mixture of molten cast iron and copper is raised for pouring into the mold may be less with the high phosphorus iron than with the low phosphorus iron. It is for this reason that a temperature range from 2300° 15 to 3000° F. has been specified in order to cover the differing characteristics of differing cast irons as to melting points and fluidity after melting.

After the composite brake drum has been cast it may be supplied with a back 21 of wrought, 20 rolled or pressed steel which is welded or otherwise suitably secured to the ring as shown in Fig. 2. The annular flask 11 is driven through the spindle 10 in any desired manner.

Having described my invention what is claimed is:

1. In a brake drum, a braking ring of cast metal comprising an inner stratum of cast iron having a circumferential bulge on its outer surface, and an outer stratum of cast copper, said copper and iron having an integrally cast connection with each other.

2. In a brake drum, a braking ring flange of centrifugally cast metals having an inner peripheral layer of cast iron and an outer peripheral layer of copper, the said iron and copper intermingling with each other forming a joinder zone of iron and copper, said joinder zone having a shape similar to the outer surface of the layer of copper.

3. A brake drum comprising a centrifugally cast annular braking member of ferrous metal having as its principal constituent iron into which is mixed copper in decreased quantity from its outer periphery inwardly, said outer periphery being a stratum of copper.

CHARLES W. DAKE.